

# United States Patent

[19]

Salesin

[11] 3,708,303

[45] Jan. 2, 1973

[54] **PHOTOGRAPHIC ELEMENTS AND PROCESSES LITHOGRAPHIC SILVER HALIDE ELEMENT CONTAINING A 1-(AMIDOPHENYL)-5-MERCAPTOTETRAZOLE SENSITIZING AGENT AND DEVELOPMENT PROCESS OF USING SAME**

[75] Inventor: Eugene D. Salesin, Rochester, N.Y.

[73] Assignee: Eastman Kodak Company, Rochester, N.Y.

[22] Filed: Jan. 12, 1971

[21] Appl. No.: 105,993

## Related U.S. Application Data

[63] Continuation-in-part of Ser. No. 754,967, Aug. 23, 1968, abandoned.

[52] U.S. Cl. 96/107, 96/109, 96/95, 96/76 R, 96/66 R, 96/33

[51] Int. Cl. G03c 5/24, G03c 1/28, G03c 5/30

[58] Field of Search 96/107, 65, 33, 109, 66, 76 R, 96/95

[56]

## References Cited

### UNITED STATES PATENTS

|           |         |                     |         |
|-----------|---------|---------------------|---------|
| 3,458,317 | 7/1969  | Ditzer et al. ....  | 96/95 X |
| 3,295,976 | 1/1967  | Abbott et al. ....  | 96/109  |
| 3,397,987 | 8/1968  | Luckey et al. ....  | 96/107  |
| 2,388,816 | 11/1945 | Bearr.....          | 96/66.1 |
| 3,025,779 | 3/1962  | Russell et al. .... | 95/94   |
| 3,128,180 | 4/1964  | Henn et al. ....    | 96/95   |

Primary Examiner—J. Travis Brown

Assistant Examiner—Won H. Louie, Jr.

Attorney—Robert W. Hampton, Bernard D. Wiese and Myron B. Kurtzman

[57]

## ABSTRACT

High contrast photographic elements comprising a support coated with a silver halide emulsion wherein the halide comprises at least about 50 mole percent chloride and containing a 1-(amidophenyl)-5-mercaptoprotetrazole, provide improved speed control without undesired change in sensitometric characteristics. Methods for processing such elements in a continuous transport processing machine are also described.

11 Claims, No Drawings

**PHOTOGRAPHIC ELEMENTS AND PROCESSES  
LITHOGRAPHIC SILVER HALIDE ELEMENT  
CONTAINING A 1-(AMIDOPHENYL)-5-  
MERCAPTOTETRAZOLE SENSITIZING AGENT  
AND DEVELOPMENT PROCESS OF USING SAME**

The application is a continuation-in-part of Ser. No. 754,967 filed Aug. 23, 1968, by Eugene D. Salesin, now abandoned.

**BACKGROUND OF THE INVENTION**

**1. Field of the Invention**

This invention relates to photographic materials, their preparation and use. One aspect of the invention relates to a continuous process for processing exposed high contrast photographic elements in a continuous transport processing machine employing photographic elements containing a 1-(amidophenyl)-5-mercaptopotetrazole. Another aspect of the invention relates to photographic emulsions containing such a 1-(amidophenyl)-5-mercaptopotetrazole, which results in desired restraining of development upon processing without undesired change in dot quality, contrast or fog of high contrast images.

**2. Description of the Prior Art**

In the graphic arts field, where it is desired to make photographic line and halftone reproductions, it is customary to employ emulsions providing extremely high contrast images. During development, the developed areas grow autocatalytically at a very high developing rate to produce extremely high contrast which is necessary for half-tone patterns and other such images requiring high dot quality. Developers utilized with lith type photographic films are quite different in composition from typical black-and-white film developers. In order to obtain very high contrast and sharp halftone dots, it has been the practice to formulate developers for such films from essentially hydroquinone, an alkaline development activator, alkali metal bromide and a low level of sulfite ion. The low level of sulfite ion partially stabilizes the developer solution for a short period of time and is achieved in all present commercial developers of this type by use of sodium formaldehyde bisulfite, which acts as a sulfite ion buffer.

Such developer solutions for high contrast lith films presently used in continuous transport processing machines have a number of disadvantages. The photographic quality obtained with a given film is usually inferior to that obtained in careful tray processing. The sensitivity of high contrast films to developer exhaustion products and development in general as well as variations in local developing agent concentration makes these films vulnerable to localized changes in sensitometric properties. For example, the dots in a high contrast film can be distorted and exhibit size changes depending on the orientation and direction of travel through the machine processor. This undesirable dot distortion is manifested in changes in the H and D curve of high contrast films which are processed in continuous transport processing machines.

Problems in the graphic arts field have also been encountered with regard to speed loss where materials are incorporated in a photographic element in an effort to improve dot quality. For example, it has been attempted in the past to incorporate 1-phenyl-5-mercaptopotetrazole in coatings for photographic elements in

order to improve dot quality. Such coatings have not proved satisfactory because an undesirable speed loss is produced which is believed to be a result of the leaching of 1-phenyl-5-mercaptopotetrazole out from the coatings. The leached out 1-phenyl-5-mercaptopotetrazole present in the developer solution would change the sensitometric properties of subsequently processed coatings. This is due to the fact that in a processing machine phenyl mercaptotetrazole gradually builds up in concentration until the entire bath must be replaced or addendum must be added to account for increased phenyl mercaptotetrazole concentrations. Accordingly, it is desirable to provide a material which satisfactorily controls speed in processing without changing any of the desired sensitometric characteristics of the coatings during machine processing.

The use of 1-phenyl-5-mercaptopotetrazole in a photographic emulsion is well known as described, for example, in U.S. Pat. No. 2,403,927 of Kendall et al. issued in 1946. The use of related compounds is also known, such as described in U.S. Pat. No. 3,266,897 of Kennard et al. issued Aug. 16, 1966, and U.S. Pat. No. 3,295,976 of Abbott and Salminen issued Jan. 3, 1967. U.S. Pat. No. 3,295,976 of Abbott and Salminen issued Jan. 3, 1967, describes the method of selectively controlling over-development of a multi-layer photographic element by a negative developer in a high temperature color process by negative development of this element in the presence of a 1-(amidophenyl)-5-mercaptopotetrazole. There is no disclosure in these patents, however, of the high contrast elements having the particular silver halide emulsions employed in the graphic arts. Moreover there is no disclosure in this patent of use of 1-(amidophenyl)-5-mercaptopotetrazole in a high contrast photographic element.

It is also known to use 1-(amidophenyl)-5-mercaptopotetrazoles as antifoggants in photographic silver halide emulsions which have fogged internal image silver halide grains and unfogged surface latent image silver halide grains as disclosed in French Pat. No. 1,492,132 of Kodak. This emulsion, however, has not been employed in high contrast photographic elements utilized in the graphic arts for producing line and halftone dot reproductions.

Accordingly, there is a need for a high contrast photographic element and process which avoids the problems resulting from leaching out of 1-phenyl-5-mercaptopotetrazole in continuous transport processing machines.

An object of the invention accordingly is to provide a high contrast photographic element containing a 1-phenyl-5-mercaptopotetrazole compound which does not significantly diffuse into processing solutions during machine processing thereby causing undesired sensitometric properties.

Another object is to provide a high contrast photographic emulsion, suitable for use in the graphic arts, which contains a non-diffusing 1-phenyl-5-mercaptopotetrazole compound.

A further object is to provide a process, especially a continuous transport process, which is suitable for developing an image in a high contrast photographic element as described.

## SUMMARY OF THE INVENTION

According to the invention, there is provided a high contrast, "lith-type" photographic element comprising a support having thereon a photographic silver halide emulsion, said halide comprising at least about 50 mole percent chloride, and said element containing a 1-phenyl-5-mercaptopotetrazole compound, especially a 1-(amidophenyl)-5-mercaptopotetrazole having the property of being non-diffusible in a high contrast photographic emulsion. In another embodiment there is provided a high contrast photographic emulsion containing a 1-(amidophenyl)-5-mercaptopotetrazole. In yet another embodiment, a continuous process is provided for processing a lith element in one continuous motion by transporting it into, through and out of at least one processing solution in the manner shown, for example, in U.S. Pat. No. 3,025,779 of Russell and Kunz issued Mar. 20, 1962; U.S. Pat. No. 3,078,024 of Sardeson issued Feb. 19, 1963; U.S. Pat. No. 3,122,086 of Fitch issued Feb. 25, 1964; U.S. Pat. No. 3,149,551 of Cramer issued Sept. 22, 1964; U.S. Pat. No. 3,156,173 of Meyer issued Nov. 10, 1963; and U.S. Pat. No. 3,224,356 of Fleisher and Hixon issued Feb. 21, 1965; wherein said element is developed in a liquid developer comprising a silver halide developing agent and a carbonyl bisulfite-amine condensation product. Such an element and process provides improved speed control without undesired change of sensitometric characteristics.

## DESCRIPTION OF THE PREFERRED EMBODIMENTS

Any 1-phenyl-5-mercaptopotetrazole which is non-diffusible in a high contrast, lith photographic emulsion and provides desired improved speed control without undesired change of sensitometric characteristics is suitable according to the invention. An especially preferred group of mercaptotetrazoles are the 1-(amidophenyl)-5-mercaptopotetrazole represented by the formula:



wherein M is an alkali metal, such as sodium, potassium or lithium, hydrogen or an organic residue, such as an organic amine residue of such amines as triethyl amine, triethanol amine, morpholine and the like; X is a radical of the formula  $-\text{SO}_2\text{R}$  or  $-\text{COR}$ , wherein R' is a hydrocarbon radical, e.g., a hydrocarbon radical containing one to 30 carbon atoms, such as alkyl, e.g., methyl, ethyl, propyl, butyl, pentyl, and eicosyl, aryl, such as phenyl or naphthyl, alkaryl, such as methylphenyl and butylphenyl and aralkyl, such as tolyl and xylyl. The hydrocarbon radical can contain various substituent groups such as alkoxy, e.g., containing one to five carbon atoms such as methoxy, ethoxy, propoxy, butoxy and pentoxy, phenoxy, halogen, cyano, nitro, amino, sulfo, sulfamyl, substituted sulfamyl, sulfonylphenyl, sulfonylalkyl, sulfonamidoalkyl, sul-

fonamidophenyl, carboxylic acid, carboxylate, carbamyl, carbamylphenyl, carbamylalkyl, carbonylalkyl, carbonylphenyl and similar groups.

Suitable 1-(amidophenyl)-5-mercaptotetrazoles include:

- 1-(3-caproamidophenyl)-5-mercaptotetrazole,
- 1-(3-pelargonamidophenyl)-5-mercaptotetrazole,
- 1-[3-(alpha-2,4-di-t-amylphenoxy)acetamidophenyl]-5-mercaptotetrazole,
- 1-(3-methylsulfonamidophenyl)-5-mercaptotetrazole,
- 1-(3-p-toluenesulfonamidophenyl)-5-mercaptotetrazole, and
- 1-(3-acetamidophenyl)-5-mercaptotetrazole.

1-(amidophenyl)-5-mercaptotetrazoles employed according to the invention can be prepared by methods known in the art such as, for example, by reaction of a corresponding 1-(aminophenyl)-5-mercaptotetrazole hydrochloride with an acid chloride of the desired amido compound. This is disclosed, for example, in U.S. Pat. No. 3,295,976 of Abbott and Salminen issued Jan. 3, 1967.

The concentration of 1-(amidophenyl)-5-mercaptotetrazole which is suitable for providing desired dot quality without loss in speed or other desired sensitometric properties, is subject to wide variation. In a photographic emulsion layer or a layer contiguous thereto, a 1-(amidophenyl)-5-mercaptotetrazole concentration of about 5 to about 275 milligrams, e.g., about 10 to about 250 milligrams per mole of silver present is suitable.

Any suitable method can be employed for incorporating the described mercaptotetrazole compounds in a photographic emulsion or layer contiguous thereto, such as mixing the described compound in a coating composition prior to the coating on a support. Any method and/or means commonly employed for incorporating addenda into photographic layers can be employed according to the invention.

The developing agents, which can be employed in processing the described photographic elements of the invention can be any of those commonly employed in the graphic arts. Useful silver halide developing agents, for example, include the dihydroxy benzenes such as hydroquinone; chlorohydroquinone; bromohydroquinone; 2,3-dichlorohydroquinone; 2,5-dimethylhydroquinone; 2,3-dibromohydroquinone; 1,4-dihydroxy-2-acetophenone-2,5-dimethylhydroquinone; 2,5-diethylhydroquinone; 2,5-di-p-phenethylhydroquinone; 2,5-dibenzoylaminohydroquinone; 2,5-diacetaminohydroquinone; etc. Esters of such compounds, for example, formates and acetates, can also be employed. These developing agents can be used alone or in any combination and can be employed in any concentration which is effective for development. A suitable concentration for the developing agent is about 0.05 to about 0.50 mole per liter of developer composition and is typically from 0.10 to about 0.30 mole per liter of developer composition.

Development activators, typically alkaline activators, are employed in the developer composition employed for processing elements of the invention. These include any of the inorganic and/or organic alkalies employed in photographic processing solutions, such as alkali metal carbonates and hydroxides, for example,

sodium hydroxide, lithium hydroxide, and potassium hydroxide, sodium carbonate, and potassium carbonate. Inorganic alkaline activators can also be employed, such as amino alkanols, for example, amino propanol, amino ethanol, diethylamine, triethylamine, iminodiethanol, etc. Any suitable concentration of development activator can be employed which provides the desired image based on the described photographic element. A concentration is employed which typically provides a developer composition having a pH well above 7, such as about 9 to about 13.

The developer compositions employed for processing the described photographic elements can also contain carbonyl bisulfite-amine condensation products, preferably formaldehyde bisulfite-amine condensation products, such as sodium-2-hydroxyethylaminoethane sulfonate; sodium-2-hydroxypropylaminomethane sulfonate; sodium-1,1-dimethyl-2-hydroxyethylaminomethane sulfonate; sodium-1,1-bis-(hydroxymethyl)ethylaminomethane sulfonate; sodium-tris(hydroxymethyl)methylaminomethane sulfonate; sodium-3-hydroxypropylaminomethane sulfonate; sodium-bis(2-hydroxyethyl)aminomethane sulfonate; sodium-N,N-bis[2-(1-hydroxy)propyl]aminomethane sulfonate; sodium-N-isopropyl-N-(2-hydroxyethyl)-aminomethane sulfonate; sodium-N-ethyl-N-(2-hydroxyethyl)-aminomethane sulfonate; and sodium-N-methyl-N-(2-hydroxyethyl)-aminomethane sulfonate. The carbonyl bisulfiteamine condensation products can be used alone or in a combination and can be employed in any concentration which is effective to provide a low level of sulfite ion in the developer composition. A suitable concentration for the carbonyl bisulfiteamine condensation product is about 0.1 to about 1.0 mole per liter of liquid developer composition and is preferably about 0.25 to about 0.50 mole per liter of liquid developer composition.

The high contrast photographic elements described according to the invention comprise a support bearing a photographic silver halide emulsion layer in which the halide comprises at least about 50 mole percent chloride. The photographic emulsions employed according to the invention are lith emulsions. Such emulsions develop to very high contrast when developed in an infectious developer. (See J.A.C. Yule "Formaldehyde-Hydroquinone Developers and Infectious Development", Jour. of the Frank. Inst., Vol. 239, No. 3, March, 1945.) A lith emulsion is typically a high contrast photographic silver halide emulsion in which the halide comprises at least 50 mole percent chloride and less than 5 mole % iodide, the remainder being bromide, said emulsion when exposed on a sensitometer and developed for 2 minutes in Kodak D-85 Developer at 20°C. having a gamma of at least 4 measured between a density of 0.3 and 3.0.

Preferably the halide in the described photographic silver halide emulsion comprises a higher concentration than about 50 percent chloride, such as at least about 85 mole percent chloride and typically at least about 90 mole percent chloride, the balance, if any, being, for example, bromide. These emulsions when exposed on a sensitometer and processed in 1 1/4 minutes through an amine developer system such as described in copending application Ser. No. 661,532, entitled,

"Photographic Developer Composition Containing Carbonyl Bisulfite Amine Condensation Product and Free Amine", filed Aug. 18, 1967 now U.S. Pat. No. 3,573,914, will have a contrast of at least about 6. Such preferred emulsions provide particularly good results in high contrast photographic elements and good dot quality. The halide of the photographic silver halide emulsion can also contain a small amount of iodide such as less than about 5 mole percent than is desired. Silver halide emulsions in which the halide comprises 100 mole percent chloride have also been found to be useful.

Other photographic elements containing lith emulsions comprising about 85 mole percent silver chloride are described in: Henn and Goffe, U.S. Pat. No. 3,030,209, issued Apr. 17, 1962, copending U.S. application Ser. No. 661,530 of Salesin entitled "High-Contrast Photographic Elements and Methods for Processing Same", filed Aug. 18, 1967, and copending U.S. application Ser. No. 661,531 of Milton, entitled "High-Contrast Photographic Elements and Methods for Processing Same" (Case A), filed Aug. 18, 1967 now U.S. Pat. No. 3,600,174.

15 The photographic silver halide emulsion layers of the high contrast photographic elements described according to the invention and/or layers contiguous thereto can contain any of the commonly employed hydrophilic water-permeable binding materials suitable for this purpose. Suitable materials include, for example, gelatin, colloidal albumin, polyvinyl compounds, cellulose derivatives, acrylamide polymers, etc. Mixtures of such binding agents can also be used. The binding agents for the described layers of the high contrast photographic elements of the invention can also contain dispersed polymerized vinyl compounds, especially those which increase the dimensional stability of photographic materials. Suitable synthetic polymers of this 20 type include, for example, water-insoluble of alkyl acrylates and methacrylates or acrylic acid. Such compounds are described for example, in U.S. Pat. No. 3,142,568 of Nottorf, issued July 28, 1964; U.S. Pat. No. 3,193,386 of White, issued July 6, 1965; U.S. Pat. No. 3,062,674 of Houck, Smith and Yudelson, issued 25 Nov. 6, 1962, and U.S. Pat. No. 3,220,844 of Houck, Smith and Yudelson, issued Nov. 30, 1965. These compounds can also be incorporated into a separate layer of the photographic element. The vinyl polymers are 30 generally employed in concentrations in the range of about 20 to about 80 percent by weight, and most often in concentrations of at least 50 percent by weight, based on the weight of the binding agent.

The described high contrast photographic elements 35 of the invention can contain an overcoat layer, such as a heavy overcoat comprising a water-permeable colloid. While any of the hydrophilic water-permeable binding materials described for the emulsion and/or other layers of the high contrast photographic element 40 can be used in the overcoat layer, gelatin has been found to produce good results. If desired the overcoat layer can also contain dispersed polymerized vinyl compounds as described.

The described high contrast photographic elements 45 of the invention can contain a photographic halide silver emulsion coated on a wide variety of supports. Hydrophilic colloid layers can be coated on one or both

sides of the support if desired. Typical supports include any of those commonly employed in preparing photographic elements for the graphic arts field such as cellulose nitrate film, cellulose ester film, polyvinyl acetal film, polystyrene film, poly(ethylene terephthalate) film and related films and/or resinous supports. Glass, paper and metal supports can also be used. Supports such as paper, which are coated with an alpha-olefin polymer, particularly polymers of alpha-olefins containing two or more carbon atoms, such as polyethylene, polypropylene, ethylene-butene copolymers and the like are suitable.

The photographic silver halide emulsions of the high contrast photographic elements of the invention can be sensitized using any of the well known techniques employed in photographic emulsion production, for example by digesting with naturally active gelatin or various sulfur, selenium, tellurium compounds and/or gold compounds. The emulsions can be sensitized with salts of noble metals of Group VIII of the Periodic Table which have an atomic weight greater than 100.

The photographic emulsions of the invention can also contain other addenda commonly employed in photographic elements used in the graphic arts such as speed increasing addenda and/or addenda for increasing contrast such as quaternary ammonium salts, polyethylene glycols, thioether sensitizers or combinations thereof. It can also contain coating aids such as anionic, nonionic and amphoteric surface active agents and the like. They also contain gelatin plasticizers, antifoggants including organic and inorganic antifoggants as well as hardeners such as aldehyde hardeners including, for example, formaldehyde, mucochloric acid, glutaraldehyde bis(sodium bisulfite), maleic dialdehyde, aziridines, dioxane derivatives and oxpolysaccharides.

The high contrast photographic silver halide emulsions of the invention can be ortho-sensitized or p-  
sensitized with spectral sensitizing dyes. For instance, these emulsions can be spectrally sensitized with merocyanine dyes, hemicyanine dyes and/or dyes useful in sensitizing such emulsions are described for example in U.S. Pat. No. 2,526,632 of Brooker and White, issued Oct. 25, 1950; and U.S. Pat. No. 2,503,776 of Sprague, issued Apr. 11, 1950.

Photographic elements according to the invention can be processed employing processing solutions and methods employed in the graphic arts and especially those employed for processing lith emulsions. They are preferably processed, typically after exposure through a contact screen employed in the graphic arts, using a 90 second development time in a Kodalith Roller Transparent 324 Film Processor of the type described in U.S. Pat. No. 3,025,779 of Russell and Kunz, issued Mar. 20, 1962, employing typically a developer having the following composition:

|                                                     |            |
|-----------------------------------------------------|------------|
| Sodium-bis-(2-hydroxyethyl)-aminomethane sulfonate* | 82.0 grams |
| Sodium sulfite                                      | 30.0 grams |
| Boric acid                                          | 7.5 grams  |
| Hydroquinone                                        | 22.5 grams |
| Potassium bromide                                   | 1.6 grams  |
| 2,2'-Iminodiethanol                                 | 39.0 grams |
| Water to make                                       | 1 liter    |
| pH                                                  | 9.5        |

Accordingly, another embodiment of the invention comprises in a continuous process for processing an exposed high contrast photographic element comprising a support coated with a photographic silver halide emulsion wherein said element is processed in one continuous motion by transporting it into, through and out of at least one processing solution, the improvement comprising the combination of:

a. developing said element in a liquid developer composition comprising a silver halide developing agent and a carbonyl bisulfite-amine condensation product,

b. said halide comprises at least about 50 mole percent chloride, and preferably at least 85 mole percent chloride, and

c. said element has a coating containing a 1-phenyl-5-mercaptopentetrazole compound having the property of being non-diffusible in a photographic emulsion. Such a process wherein the 1-phenyl-5-mercaptopentetrazole

compound is a 1-(amidophenyl)-5-mercaptopentetrazole, as described, is preferred. A process of the invention is also preferred wherein the developer solution is an aqueous solution containing a hydroquinone developing agent in a concentration of about 0.05 to about

0.50 mole per liter of solution and containing a formaldehyde bisulfite-amine condensation product present in a concentration of about 0.10 to about 1.0 mole per liter of developer solution.

Typically the processed element of the invention, as employed in the graphic arts field, consists of a pattern of dots, areas commonly referred to as shadow dots and areas known as high-light areas. Intermediate between the two extremes of areas referred to as shadow dots and areas known as high-light areas are areas of varying size. The common method in the graphic arts for measuring the quality of reproduction of a photographic element is to examine the dot areas. The quality of dot can be expressed on any convenient scale, but for the purposes of the invention the following scale can be employed to refer to a quality of dot: a grade scale between 1 and 9 is employed wherein 9 is excellent and 1 is extremely poor with varying degrees of quality between these two points. This scale is employed herein to designate the quality of image.

The following examples are included for a further understanding of the invention.

#### EXAMPLE 1

A fine-grain silver chlorobromoidide gelatino emulsion containing 90 mole percent chloride, 9 mole percent bromide and 1 mole percent chloride is chemically sensitized with sulfur and gold compounds and coated on a polyethylene terephthalate support. The emulsion is applied to the support at the rate of 456 milligrams of silver per square foot, 296 milligrams of gelatin per square foot and 296 milligrams per square foot of alkyl acrylate polymer as described in U.S. application Ser. No. 525,272 filed Dec. 20, 1965 of D. A. Smith now U.S. Pat. No. 3,459,798. A gelatin overcoat is coated on the resulting emulsion layer at 82.6 milligrams per square foot. The resulting product is designated as Product A and employed as a control.

Identical coatings are made with the exception that 1-(3-acetamidophenyl)-5-mercaptopentetrazole, also known as AcPMT, is added to separate portions of the described emulsion at the rate respectively of 5, 25 and

125 milligrams of 1-(3-acetamidophenyl)-5-mercaptopotetrazole per mole of silver present. These products are designated, respectively, as Product B, Product C and Product D.

The resulting dried coatings are exposed using tungsten illumination to a step wedge through a magenta contact screen. The element are then processed using a 90 second development time in a Kodalith Roller Transport 324 Film Processor as described in U.S. Pat. No. 3,025,799 of Russell and Kunz, issued Mar. 20, 1962 employing the following developer:

|                                                     |            |
|-----------------------------------------------------|------------|
| Sodium-bis-(2-hydroxyethyl)-aminomethane sulfonate* | 82.0 grams |
| Sodium sulfite                                      | 30.0 grams |
| Boric acid                                          | 7.5 grams  |
| Hydroquinone                                        | 22.5 grams |
| Potassium bromide                                   | 1.6 grams  |
| 2,2'-Iminodiethanol                                 | 39.0 grams |
| Water to make                                       | 1 liter    |
| pH                                                  | 9.5        |

\*Sodium formaldehyde bisulfite and 2,2'- iminodiethanol can be used to form this compound in situ.

The resulting image consists of a pattern of dot areas commonly referred to in the art as shadow dots and areas known as high-light areas. Intermediate between these two extremes are areas of varying size including a so-called middle tone area. The letters H, M and S described herein refer respectively to high-light, middle tone, and shadow dots.

The results obtained are set out in Table I. The relative speed, effective contrast and dot quality are given for varying development time. Development time is varied between 1 1/2 minutes, i.e. 90 seconds, and 2 1/4 minutes, i.e., 135 seconds.

TABLE I

| Product          | AcPMT,<br>mg./Ag<br>mole | Relative speed |        |     |        | Effective contrast |        |     |        | Dot quality |             |         |             |
|------------------|--------------------------|----------------|--------|-----|--------|--------------------|--------|-----|--------|-------------|-------------|---------|-------------|
|                  |                          | 1 1/2'         | 1 3/4' | 2'  | 2 1/4' | 1 1/2'             | 1 3/4' | 2'  | 2 1/4' | 1 1/2'<br>M | 1 3/4'<br>H | 2'<br>M | 2 1/4'<br>S |
| A (control)..... | None                     | 100            | 141    | 155 | 166    | 7.7                | 8.5    | 9.0 | 9.0    | 7           | 484         | 8       | 8           |
| B.....           | 5                        | 100            | 132    | 138 | 149    | 7.7                | 8.8    | 9.0 | 9.0    | 8           | 484         | 8       | 8           |
| C.....           | 25                       | 68             | 87     | 100 | 110    | 7.5                | 7.4    | 7.6 | 8.0    | 8           | 484         | 8       | 8           |
| D.....           | 125                      | 40             | 53     | 55  | 65     | 7.3                | 7.6    | 7.5 | 8.0    | 8           | 484         | 8       | 8           |

Results in Table I illustrates that even change in relative speed is obtained for each concentration level of 1-(3-acetamidophenyl)-5-mercaptopotetrazole with no change in dot quality and no appreciable change in effective contrast. Effective contrast is the average gradient of the density versus Log E curve between two points, which are 0.3 Log E apart where the lower point has a density of 0.1 above fog. It is measured as the slope of a straight line between these points. Fog is 0.01 for all described coatings and processing times.

## EXAMPLE 2

This is a comparative example illustrating advantages of the invention.

Four photographic elements are prepared as set out in Example 1 and are designated respectively as Products E, F, G, and H. These products contain the following differences from the products described in Example 1:

E. Product E contains no 1-(3-acetamidophenyl)-5-mercaptopotetrazole or 1-phenyl-5-mercaptopotetrazole.

F. Product F contains 125 milligrams of 1-phenyl-5-

mercaptopotetrazole in place of 1-(3-acetamidophenyl)-5-mercaptopotetrazole per mole of silver.

G. Product G contains 125 milligrams of 1-(3-acetamidophenyl)-5-mercaptopotetrazole per mole of silver.

H. Product H contains 250 milligrams of 1-(3-acetamidophenyl)-5-mercaptopotetrazole per mole of silver.

500 milliliter portions of the developer solution described in Example 1 are employed. Fifteen unexposed 4 × 10 inch sheets (4.15 square feet) of each of the described Products E, F, G and H are passed through the described developer portions. The resulting developer is designated as Developer A. Then 30 unexposed 4 × 10 inch sheets (8.30 square feet) of Products E, F, G, and H are passed through separate 500 milliliter portions of the developer composition set out in Example 1. The resulting developer is designated as Developer B.

A control, as described in Example 1, containing neither phenylmercaptopotetrazole or 1-(3-acetamidophenyl)-5-mercaptopotetrazole is prepared and exposed as set out in Example 1. The resulting element is processed for 1 1/4 minutes, i.e., 105 seconds, at 27°C. in each of the resulting developer solutions, i.e., each of Developer A and Developer B. The results of these tests are compared to the control processed in a fresh developing solution whose speed is assigned 100.

25 The results are also compared to the control processed in a fresh developing solution to which is added 8.72 milligrams of 1-(3-acetamidophenyl)-5-mercaptopotetrazole per 500 milliliters of developing solution. (8.72 milligrams of 1-(3-acetamidophenyl)-5-merc-

30 The results are also compared to the control processed in a fresh developing solution to which is added 8.72 milligrams of 1-(3-acetamidophenyl)-5-mercaptopotetrazole per 500 milliliters of developing solution. (8.72 milligrams of 1-(3-acetamidophenyl)-5-merc-

| Product          | AcPMT,<br>mg./Ag<br>mole | Relative speed |        |     |        | Effective contrast |        |     |        | Dot quality |             |         |             |
|------------------|--------------------------|----------------|--------|-----|--------|--------------------|--------|-----|--------|-------------|-------------|---------|-------------|
|                  |                          | 1 1/2'         | 1 3/4' | 2'  | 2 1/4' | 1 1/2'             | 1 3/4' | 2'  | 2 1/4' | 1 1/2'<br>M | 1 3/4'<br>H | 2'<br>M | 2 1/4'<br>S |
| A (control)..... | None                     | 100            | 141    | 155 | 166    | 7.7                | 8.5    | 9.0 | 9.0    | 7           | 484         | 8       | 8           |
| B.....           | 5                        | 100            | 132    | 138 | 149    | 7.7                | 8.8    | 9.0 | 9.0    | 8           | 484         | 8       | 8           |
| C.....           | 25                       | 68             | 87     | 100 | 110    | 7.5                | 7.4    | 7.6 | 8.0    | 8           | 484         | 8       | 8           |
| D.....           | 125                      | 40             | 53     | 55  | 65     | 7.3                | 7.6    | 7.5 | 8.0    | 8           | 484         | 8       | 8           |

45 totetrazole is calculated as the approximate amount that is leached out under equilibrium conditions for processing coatings containing 125 milligrams of 1-(3-acetamidophenyl)-5-mercaptopotetrazole per mole of silver).

50 The following Table II lists the results obtained. Table II lists the relative speeds of the control coating processed in developing solutions through which were passed the described 4 × 10 inch sheets of Products E, F, G and H.

TABLE II

| Control     | prior art<br>Prod. F<br>Prod. E<br>None | invention<br>Prod. G<br>125 mg.<br>PMT/mole | invention<br>Prod. H<br>250 mg.<br>AcPMT/<br>mole |
|-------------|-----------------------------------------|---------------------------------------------|---------------------------------------------------|
| Developer A | 102                                     | 94                                          | 101                                               |
| Developer B | 94                                      | 53                                          | 99                                                |

65 The relative speed of the control coating when employing a fresh developer containing 8.72 milligrams of 1-(3-acetamidophenyl)-5-mercaptopotetrazole is 76, whereas the relative speed of a control containing no

mercaptotetrazole compound is 100.

A comparison of the relative speeds of each of the coatings listed in Table II illustrates that:

a. 1-(3-acetamidophenyl)-5-mercaptotetrazole, when added to the described developing solution, provides a speed loss for coatings processed therein;

b. photographic elements according to the invention containing 1-(3-acetamidophenyl)-5-mercaptotetrazole provide no speed loss, thus indicating that the described mercaptotetrazole of the invention does not leach out of the described coating; and

c. there is a speed loss for the control processed in a developer solution in which coatings containing 1-phenyl-5-mercaptotetrazole are previously processed. This indicates that, surprisingly, by employing a photographic element of the invention the disadvantageous sensitometric effects caused by employing a photographic element containing 1-phenyl-5-mercaptotetrazole are avoided.

The invention has been described in detail with particular reference to preferred embodiments thereof, but it will be understood that variations and modifications can be effected within the spirit and scope of the invention.

I claim:

1. A high contrast photographic element comprising a support having thereon a photographic lith type silver halide emulsion wherein said halide comprises at least about 85 mole percent chloride, said element containing a 1-(amidophenyl)-5-mercaptotetrazole, said mercaptotetrazole being nondiffusible in a photographic emulsion.

2. A high contrast photographic element as in claim 1, wherein said 1-(amidophenyl)-5-mercaptotetrazole compound is present in a coating contiguous to said photographic silver halide emulsion.

3. A high contrast photographic element as in claim 1 wherein said mercaptotetrazole is a 1-(3-acetamidophenyl)-5-mercaptotetrazole.

4. A high contrast photographic element as in claim 1 containing about 5 to about 250 milligrams of said 1-(amidophenyl)-5-mercaptotetrazole per mole of silver present in said photographic silver halide emulsion.

5. A high contrast photographic lith silver halide emulsion, said halide comprising at least about 85 mole

percent chloride, containing about 5 to about 250 milligrams of a -(amidophenyl)-1-(aminophenyl)-5-mercaptotetrazole per mole of silver, said mercaptotetrazole being nondiffusible in a photographic emulsion.

6. A high contrast photographic lith type silver halide emulsion as in claim 5 wherein said halide comprises about 90 mole percent chloride, about 1 mole percent iodide and about 9 mole percent bromide.

7. In a continuous process for processing an exposed high contrast photographic element comprising a support coated with a photographic lith type silver halide emulsion, said process comprising the steps of transporting said element in one continuous motion into, through and out of at least one processing solution comprising a liquid developer composition, the improvement comprising the combination of:

- a. said developer composition comprising a silver halide developing agent and a carbonyl bisulfite-amine condensation product,
- b. said halide comprising at least about 85 mole percent chloride, and
- c. said element having a coating containing a 1-(amidophenyl)-5-mercaptotetrazole being nondiffusible in a photographic emulsion.

8. A process as in claim 7 wherein said 5-mercaptotetrazole is 1-(3-acetamidophenyl)-5-mercaptotetrazole.

9. A process as in claim 7 wherein said developing agent is a dihydroxybenzene developing agent and said carbonyl bisulfite-amine condensation product is a formaldehyde bisulfite-amine condensation product.

10. The process of claim 7 wherein said developer solution is an aqueous solution, said developing agent is hydroquinone present in said solution in a concentration of about 0.05 to about 0.50 mole per liter of developer solution and said carbonyl bisulfite-amine condensation product is a formaldehyde bisulfite-amine condensation product present in a concentration of about 0.10 to about 1.0 mole per liter of developer solution.

11. The process of claim 7 wherein said photographic element is transported by rollers.

\* \* \* \* \*